# EUROPEAN PATENT SPECIFICATION

(11) **EP 0 719 978 B1**
(45) Date of publication and mention of the grant of the patent: **24.10.2001**
(21) Application number: 95402914.6
(22) Date of filing: 22.12.1995
(51) Int. Cl.: F17C 9/00

(54) **A process for distributing ultra high purity gases with minimized corrosion**
Verfahren zum Verteilen von ultrareinen Gasen mit minimierter Korrosion
Procédé pour distribuer des gaz à ultra haute pureté avec corrosion minimisée

(30) Priority: 30.12.1994 US 366468; 25.07.1995 US 506867
(43) Date of publication of application: 03.07.1996
(73) Proprietor: L'AIR LIQUIDE, SOCIETE ANONYME POUR L'ETUDE ET L'EXPLOITATION DES PROCEDES GEORGES CLAUDE, 75321 Paris Cédex 07 (FR)
(72) Inventor: Kimura, Masao, Tsuchiura-shi, Ibaraki 300 (JP); Tsukamoto, Toshiyuki, Ushiki-shi, Ibaraki-pref.300-12 (JP); Tarutani, Kohei, Tsukuba-shi, Ibaraki 305 (JP); Friedt, Jean-Marie, Chuo-ku, Tokyo 104 (JP)
(74) Representative: Vesin, Jacques

(56) References cited:
- EP-A- 0 392 985
- US-A- 4 723 363
- JOURNAL OF VACUUM SCIENCE AND TECHNOLOGY: PART A, vol. 11, no. 4, PART 02, 1 July 1993, pages 1719-1724, XP000403685 TATENUMA K ET AL: "QUICK ACQUISITION OF CLEAN ULTRAHIGH VACUUM BY CHEMICAL PROCESS TECHNOLOGY"

## Description

### FIELD OF THE INVENTION

The present invention relates to the distribution of ultra high purity electronic specialty gases. More particularly, the present invention relates to the minimization of corrosion in the distribution of ultra high purity gases.

### BACKGROUND OF THE INVENTION

The use of ultra high purity of chemicals, in particular of chemical gases, used in the processing of electronic materials is known to be a key factor in achieving acceptable production yield, production reproducibility and high quality in the manufacturing of electronic devices. For a recent review, see e.g., M. Liehr and G.W. Rubloff, J. Vac, Sci, Technol. B 12, 2727 (1994).

Even if high purity is achieved at the manufacturing and purification step of such chemical gases, it is known that contamination occurs easily during their transportation to the point of use, through an equipment network (also referred to as a gas distribution network) which can include large lengths of tubing and many components for the control of pressure and flow rate (e.g. pressure reducers, valves, mass-flow controllers, filters, purifiers, etc.) which have to be interposed in a wafer fabrication between the source (e.g. gas cylinders) and the point of use (e.g. the process reactor) as well as other components well known to those of ordinary skill in the art.

The problem is of particular concern in the case of corrosive gases, such as halogen containing gases, which easily react with exposed surfaces including the communication surfaces of the gas distribution network through corrosion reactions. Such corrosion reactions may generate not only particulate contamination but also completely modify the adsorption-desorption properties of the gas and its impurities on the thus modified surface. Ultimately, corrosion phenomena may create leakage or malfunction of mobile parts, which will be of concern with respect to the safety efficiency and effectiveness of the gas distribution equipment.

Such corrosion reactions are known to be associated with the presence of moisture, even in minute quantities. Although state of the art corrosive gases are very pure with an H₂O concentration typically below 1 ppm (1 part per million) [See e.g. Miyazaki et al., Bull. Chem. Soc. Japan 66, 3508(1993); 66, 969(1993)], the corrosion reactions often take place by mechanisms involving the moisture adsorbed on the communication surface of a gas distribution network.

The current objective in purity of ultra clean electronic specialty gases to be delivered at point of use is in the range of 1 to 100 ppb (parts per billion) for any volatile impurity, particulate density lower that 1 particulate per cubic foot (under normal condition) and metal concentrations of less than 100 ppt (parts per trillion) for any metallic element present.

A major mechanism of microcontamination in the above considered purity range arises from the difficulty of completely removing adsorbed molecules from the surface of the materials exposed to the electronics specialty gases, and in particular of moisture, which is widespread in the environment and presents a particularly strong adsorption energy to surfaces.

Many of the corrosion electronic specialty gases, although of high purity, i.e., with less than 1 ppm H₂O concentration, tend to react with such adsorbed molecules, particularly H₂O adsorbed on metallic surfaces, though a catalytically activated chemical reaction, which promotes corrosion and the formation of volatile or solid by-products in the considered concentration range and also solid particulates.

The usual procedure carried out to clean such a gas distribution network is to flow ultra high purity inert gas (e.g. nitrogen or argon of purity better than 1 ppb) in order to purge all impurities present in the volume or at the communication surfaces of the gas distribution network. This procedure is nevertheless unsatisfactory for strongly adsorbed molecules, e.g. H₂O molecules adsorbed on solid surfaces. Others have attempted to improve this purge procedure and reduce its duration by using successive pressure-vacuum cycles of the inert gas and also by heating the surface in order to induce thermal desorption of the strongly adsorbed molecular species. However, these vacuum-pressure purge cycles prove inefficient in locations representing deep deadspaces because of the inefficiency of pumping through minute orifices.

Still others have attempted thermal baking at 120°C during the purge of metallic surfaces. Such a procedure is known to significantly reduce the time to reach the background level of the purge gas. For example, one can obtain 1 ppb purity in a few hours when flowing ultra high purity (<1 ppb impurity) nitrogen or argon at 0.1-10 standard liter per minute through a gas distribution network free of microleaks of a length between about 10 and about 200 meters, approximately. However, it is also known that the thermal desorption of H₂O on an electropolished stainless steel surface occurs in several steps, the last one being at temperature of the order of 400°-450°C. Such a temperature is difficult to apply in practice. Hence, when lower baking temperatures are applied, e.g. frequently 120°C for practical reasons, the metal surface is not entirely free of adsorbed moisture. Moreover, thermal baking cannot be applied in practice under some circumstances for safety, regulation or material stability reasons.

Others have attempted to improve the purge procedure of the gas distribution network, using for instance a larger number of vacuum-pressure cycles, or increasing the flow rates of the ultra high purity gases. Although this may decrease the initial concentration of the generated impurities and particulates, the time required to reach the background level is always quite long, i.e. about 40 minutes at 40 sccm flow rate and about 15 minutes at 30 sccm flow rate.

Others have used chemical-drying agents in the vapor phase such as DMP (acetone dimethyl acetal), DCP (2-2-di-chloropropane or DBP (di-bromopropane) as has been reported where they react with adsorbed moisture (K. Tatenuma et al., J. Vac. Sci. Technol. All, 1719 (1993); K.Tatenuma et al., Bunseki 223, 393 (1994) or also as liquid mixed with fluorocarbon liquids (Kokai, 5-140777).

The wet cleaning removes molecular species soluble in these liquids or removes by dilution or liquid mechanical friction molecular species and particulates which may reside on the surfaces before the below described wet drying. Thus, wet cleaning of the gas communicating surfaces of the various components of the gas distribution network removes surface impurities (molecules or particulates).

Surface modifications induced by corrosion will affect the adsorption energy between the surface and both the Electronic Speciality Gas (ESG) and its impurity, hence resulting in a gas of fluctuating composition at the point of usage. Moreover, in the operation of such a gas distribution network, it is essential to prevent the intrusion of any moisture or air, or to be able to remove the resulting intruded molecules if this should happen.

It is therefore an object of the present invention to provide another technology to more effectively dry the surfaces, particularly for deep deadspace locations or those which cannot be heated for thermal desorption because of practical, hazardous or regulatory conditions.

It is also an object of the present invention to provide a process to remove adsorbed molecules, particularly H₂0, before introducing electronic specialty gases into a distribution network, in an effort to suppress the above-described source of corrosion and of microcontamination by volatile or particulate impurities.

It is a further object of the present invention to provide a process for minimizing corrosion in the distribution of ultra high purity gases.

It is further an object of the present invention to provide a process for the minimization of contaminants and particulates generated by corrosion in the distribution of ultra high purity gases.

### SUMMARY OF THE INVENTION

The foregoing objectives are achieved by a process for reducing corrosion in a gas distribution network of ultra high purity gas or any part thereof, comprising:
(a) Wet cleaning the gas distribution network or at least one part thereof with a wet cleaning agent; and
(b) Liquid drying said gas distribution network or said at least one part thereof with an H₂O desorbing liquid drying agent selected from the group consisting of acetone dimethylacetal (equivalently called dimethoxy propane) (DMP), 2.2 dichloropropane DCP or 2.2 dibromopropane DBP, mixtures thereof and any equivalent thereof.

### BRIEF DESCRIPTION OF THE DRAWINGS

Figure 1a and 1b illustrate two different apparatus for carrying out the process of the present invention.

Figure 2 is a graph that depicts particulates emitted from a gas cylinder through a cylinder valve.

Figure 3 is a graph that depicts particulates emitted from a gas cylinder through a cylinder valve which has been liquid dried according to the present invention.

Figure 4 is a comparative graph that depicts total metals leached on DI water of the HBr cylinder valve before and after the liquid drying of the present invention.

Figure 5 is a comparative graph that depicts total metals leached on DI water rinsing of the DCS cylinder valve before and after the liquid drying of the present invention.

### DETAILED DESCRIPTION OF THE PREFERRED EMBODIMENTS

The process of the present invention includes:
(a) Wet cleaning the gas distribution network or at least one part thereof with a wet cleaning agent; and
(b) Liquid drying said gas distribution network or said at least one part thereof with an H₂O desorbing liquid drying agent selected from the group consisting of acetone dimethylacetal DMP, 2.2 dichloropropane DCP or 2.2 dibromopropane DBP, mixtures thereof and any equivalent thereof.

The present invention provides for the corrosion reduced distribution of ultra high purity gases based on the improved removal of moisture adsorbed on metal surfaces and other surfaces comprised.

The process of the present invention is particularly well suited for the problem of corrosion originating from a cylinder valve since thermal desorption of the species adsorbed in the cylinder valve is prevented by safety and regulation considerations.

The present invention includes wet cleaning at least a portion of a gas distribution network which is the most corrosion sensitive (such as valves), liquid drying of at least said portions of the gas communicating surfaces of the gas distribution network through exposure to an H₂O desorbing liquid drying agent which reacts with adsorbed moisture and preferably leaves neither substantial particulate residues nor substantial volatile molecules adherent to the metal surface. The liquid drying of the present invention can be completed very effectively at room temperature using a liquid chemical which preferentially removes adsorbed H₂O and which will leave neither particulate residue nor volatile molecules presenting strong interaction energy to the surface. The latter are hence easily purged out under vacuum-pressure cycles after the liquid drying step.

In one embodiment of the present invention such liquid drying agents include DMP (Acetone Dimethyl Acetal), DCP (2-2-Dichloropropane) or DBP (DiBromopropane). However, other H₂O desorbing liquid drying agents known to those of ordinary skill in the art can be used in accordance with the present invention. It is most preferred to use pure liquids, in order to combine the wet cleaning and drying properties of these molecules.

Preferably thereafter, purging of any residual by-product is accomplished, preferably by pressure-vacuum cycle purge using ultra high purity inert gas, preferably dry and preferably containing less than 1 ppm of any impurity. Then an evacuation step is preferably carried out at a pressure which is preferably lower than 5 x 10⁴ Pascal. The above procedure is done before exposing said surfaces to the electronic specialty gas, particularly the corrosive ones like HBr, or the like, or ambient air.

The wet-cleaning by a high purity liquid, e.g. DI water, alcohols, acetone or others, removes molecular species soluble in these liquids. It also removes by dilution or liquid mechanical friction molecular species and particulates which may accidentally reside on the gas communicating surfaces before the above described wet drying.

This step is particularly useful when the gas distribution network or any part thereof is accidentally exposed to air, e.g. during cylinder connection or opening the network for repair or component exchange, moisture will be adsorbed on the surfaces. The presence of adsorbed H₂O will promote corrosion reactions. The detrimental effect of such accidental corrosions can be effectively substantially suppressed by the above-described combination of the wet cleaning step prior to the liquid drying step (with or without purging with high purity inert gas or with or without vacuum pressure cycles between wet cleaning and liquid drying).

In another embodiment of the present invention, the same wet cleaning and liquid drying procedure is preferably also applied just after purging the ESG from an exposed component and before exposing it, even very briefly, to air. This is done in order to suppress the unwanted corrosion which may arise by reaction between residual adsorbed ESG and H₂O molecules, which will occur after air exposure. Indeed, such reactions between adsorbed species are again catalytically activated and promote surface reaction leading to corrosion, particulates and formation of unwanted surface molecules.

In yet another embodiment of the present invention, repeated cycles of wet cleaning and liquid drying are completed. This sequence is particularly effective before and after any exposure of a surface to an ESG, particularly when the surface has been exposed to air.

Among the many appropriate uses for the process of the present invention, particularly the combination of steps (a) and (b), it is intended for use before (a) any exposure (even for a minimal time) to air and (b) before flowing the ESG through the gas distribution network.

The present invention provides a procedure for corrosion reduced or free, i.e. volatile reaction byproducts-reduced and particulates-reduced, electronic specialty gases distribution based on the improved removal of moisture adsorbed on metal surfaces and other surfaces. The process of the present invention is particularly well suited for the problem of corrosion originating from a cylinder valve since thermal desorption of the species adsorbed in the cylinder valve is prevented by safety and regulation considerations.

The process of the present invention may optionally first include purging said distribution network or any part thereof with a dry inert high purity gas comprising preferably less than 1 ppm of any impurity and more particularly less than 1 ppm water vapor. After purging and venting the purging gas, then the distribution network is usually evacuated to sub-ambient pressure. These two first steps may be repeated until a pressure of less than 5 x 10⁴ Pascal is reached, with an impurity content in the gas vented which is similar to that of the inert gas injected to purge. These steps (repeated as many times as necessary) are known as "cycled pressure-vacuum" purging. After these two optional steps, the gas distribution network is wet cleaned and liquid dried as indicated hereabove. The wet cleaning is accomplished with a high purity liquid such as DI water, alcohols, acetone or other similar cleaning agents known to those of skill in the art. The wet cleaning agents used in this step of the process according to the invention shall be high purity cleaning agents suitable for cleaning metallic surfaces, particularly stainless steel surfaces. By high purity, it is meant cleaning agents which, when they are used pure (or in admixture with other cleaning agents or solvents) do not leave substantial solid residues on the treated surface, i.e. comprising less than 1 mg. of solid residue per liter and preferably less than 10⁻⁶ g of solid residue per liter.

The injection of the wet cleaning (liquid) agent is made by any appropriate means such as disclosed hereafter with Figure 1a and 1b. This injection can be done either manually with a syringe or automatically with a pump through capillary tubes.

The duration of this wet cleaning step is usually between about 1 min. to at most 1 hour. If the pipes and other components are new (i.e. have never been used before), it is usually not necessary to wet clean them. However, if it is believed that some particles or condensible molecules may have already adhered, wet cleaning during about 1 min. to about 2 min. is sufficient. If the pipe distribution network and/or other components of the network have already been used before, it is usually recommended to clean them between about 5 to about 30 min., preferably about 10 min.

Of course, this cleaning is applicable to pipings, valves, mass flow controllers and the like. As a new or existing gas distribution network, it is advisable to provide the process according to the invention each time, as an internal surface of the network shall be in contact with air. For example, when a cylinder is filled in a plant with an electronic specialty gas, it is recommended to clean/dry the valve as explained in the present specification at the end of the filling step. When the cylinder is delivered in the plant of the customer, it is also recommended to apply to said valve of said cylinder the process as disclosed in this specification particularly steps (a) and (b). Also, when the cylinder is withdrawn from the gas cabinet when it is empty, the same procedure should apply. Purging with inert gas between the wet cleaning step (a) and the liquid drying step (b) is usually optional.

The wet cleaning step (a) is then followed by a step comprising a liquid drying of the gas communicating surfaces of the gas distribution network through exposure to chemicals which react with adsorbed moisture and leave neither particulate residues nor volatile molecules adherent to the metal or other surface. This wet-drying step is intended to prevent any catalytic reaction of decomposition by water of the electronic specialty gases which flow through the distribution network. Liquid drying according to the present invention can be effectively completed at room temperature using a liquid chemical which preferably removes adsorbed H₂O and which will leave neither particulate residue nor volatile residue (liquid/vapor) but being chemically active with adsorbed moisture. (No particulate residues means that the liquid contains usually less than 1 mg and preferably less than 10⁻⁶/g of particulate material per liter). These liquid chemicals are hence easily purged out under vacuum-pressure cycles after the liquid drying.

The duration of this liquid drying step is preferably between about 1 min. to about 20 minutes. Usually, if the device or piping distribution network is new and the roughness of the internal surface of the same is less than 5 x 10⁻⁶m (Ra< 5 x 10⁻⁶m), about 1 to about 2 minutes are usually enough. However, if the device, piping or network are not new and/or if the roughness of the surface Ra is greater than 5 x 10⁻⁶m, then it is usually recommended to treat with the drying agent during about 10 minutes or more.

According to the invention, the H₂O desorbing liquid drying agent is selected from the group consisting of DMP (acetone dimethyl acetal), DCP (2-2-di-chloropropane) or DBP (2-2 dibromopropane), any mixture thereof and any equivalents thereof. An equivalent is herein defined as any liquid which can react with adsorbed moisture and leaves neither substantial particulate residues nor substantial volatile molecules adherent to the metal or other surface and which function is to prevent any catalytic reaction of decomposition by water of the electronic specialty gases which flow through the distribution network. It is most preferred to use pure liquids, in order to combine the wet-cleaning properties and chemical-drying properties of these molecules.

According to one aspect of the present invention, it has been unexpectedly discovered that the three above drying liquids (DMP, DCP or DBP), when used after the wet cleaning step disclosed hereabove, were extremely effective and that it cannot be accurately predicted whether other molecules of other H₂O desorbing liquid drying agent can be used as much successfully. However, it is well within the skills of the man skilled in the art to try another H₂O desorbing liquid to determine whether they are suitable or not.

Usually thereafter, purging of any residual by-product is accomplished preferably by pressure-vacuum cycle purge using ultra high purity inert gas, comprising preferably less than 1 ppm of any purity.

In an especially preferred embodiment of the present invention, the gas distribution network is purged with an inert gas such as nitrogen, argon, helium or with a reductive gas such as hydrogen, after the wet cleaning and liquid drying steps have been completed and before the delivery of the ESG. The duration of purging may vary between about 1 minute to about 10 minutes, preferably between 2 to 5 minutes. The gas used for such purging has to be of course extremely pure, i.e. less than bout 100 ppb of volatile impurities and less than one particle per liter in normal conditions of temperature and pressure. (This purging with the above gases is usually carried out with alternate vacuum).

Next, an ESG is introduced into the gas distribution network. For the purpose of the present invention, an ESG means a corrosive gas or an electronic specialty gas which may have some corrosive properties or suspected corrosive properties. Also, of course, gas distribution network, or parts thereof which are essentially treated as disclosed hereabove, whether used to flow corrosive gas or any other gas (such as N₂). The present process essentially comprises the various treatment steps to reduce corrosion, whether or not a corrosive gas is further flown in the gas distribution network.

In another embodiment of the present invention, after flowing the ESG for the manufacturing process, such as I.C. manufacturing, the wet cleaning and the liquid drying steps (a) and (b) of the present invention are additionally performed just after purging the ESG from the distribution network and before exposing the network, even very briefly, to air. This reduces the occurrence of unwanted chemical reaction between residual adsorbed ESG and H₂O molecules, which will occur after air exposure. Indeed, such reactions between adsorbed species are again catalytically activated and promote surface reaction leading to corrosion.

In yet another embodiment of the present invention, two cycles or more of wet cleaning (e.g. the first using e.g. Di water--less volatile--the second using e.g. acetone or alcohol--more volatile) and at least one cycle of wet drying are completed. This sequence is particularly effective both before and after any exposure of a gas communicating surface of the gas distribution network to an ESG, particularly when the surface has been exposed to air.

Among the many appropriate uses for the process of the present invention, it is intended for use before (a) any exposure (even for a minimal time) to air and (b) before flowing the ESG through the gas distribution system or any part thereof.

The above process can be applied to a total gas distribution network. However, the most critical parts are those involving deep deadspaces such as found in a valve construction or other components such as mass flow controllers, pressure regulators, etc. Accordingly, the present invention is specially directed to such components in the gas distribution network.

A gas distribution network capable of carrying out the wet cleaning and/or liquid drying step of the present invention is rather intricate because of the deadspaces involved in a valve construction. Accordingly, the present invention is also directed to a gas distribution network capable of carrying out the process of the present invention with minimal deadspace.

An apparatus for carrying out the process of the present invention includes a means for wet cleaning the gas distribution network and a means for liquid drying the gas distribution network with an H₂O desorbing liquid agent.

According to one embodiment of the apparatus of the present invention, the wet cleaning and/or liquid drying agent can be introduced to the gas distribution network manually using a syringe type introduction system as represented on Figure 1a and 1b.

In a preferred embodiment of the apparatus of the present invention, the circulation of the wet cleaning and/or liquid drying agents is achieved by the use of capillary tubing and includes the use of a circulation pump as a preferred method of operation as depicted in Figure 1a. The apparatus of Figure 1a provides a mechanically activated liquid circulation system designed to reach deep deadspaces within the components of the gas distribution network in implementing the process of the present invention. The system is based on a pump to provide liquid flow, capillary inlet and outlet lines to provide minute deadspaces and an assembly allowing clean fluid handling and minimal air exposure on connection and disconnection. The apparatus of Figure 1a is further described below.

The cylinder valve head assembly of Figure 1a includes a cylinder valve 1, diaphragm 2, spring 3, spindle 4, polymeric sealing material such as Diflon, Teflon or others 5, cylinder valve port 6, gas flow from cylinder 7 (for example HBr), outlet of cylinder valve 8, polymeric packing 9 and fitting and connector 10.

The cylinder valve head assembly is in fluid communication with a length of capillary tubing 11 and a first end of a "T" type male connector 12. A first end of a three-way diaphragm valve for wet cleaning and/or liquid drying inlet 20 is in fluid communication with a second end of the "T" type male connector 12. We use ceramic cement as a vacuum-tight, non-reactive and non-outgasing metal-metal bonding agent.

A liquid pump 24 is in fluid communication with a second end of the three-way diaphragm valve for wet cleaning and/or liquid drying inlet 20. Liquid pump 24 is further in fluid communication with a 0.1 *µ*m filter 26 and wet cleaning agent or liquid drying agent 25.

A third end of the three-way diaphragm valve for wet cleaning and/or liquid drying inlet 20 is in fluid communication with diaphragm valve 21 which is in further communication with 0.1 *µ*m filter 22 and dry gas inlet 23. Dry gas inlet 23 is used for the introduction of purge gases (inert or reductive, usually used between the cleaning step and the drying step).

A third end of the "T" type male connector 12 is in fluid communication sequentially with a three-way diaphragm valve for evacuation 14 by oil free vacuum pump 19, a three-way diaphragm valve 15 for moisture monitor by hygrometer 18, a diaphragm valve 16 and a vent line 17 for wet cleaning and/or liquid drying which is connected to recovering means (not shown in the drawing) to recover those products after being used.

In operation, the apparatus of Figure 1 is operated as follows:
1. Close cylinder valve;
2. Open valve 16, close valve 14, 15, 20 and 21;
3. Insert capillary tubes into cylinder valve;
4. Connect apparatus to cylinder valve outlet (8) by the connector (10);
5. Open valve 20 and switch on the pump (24) (automatic) or a syringe (manual), and send cleaning liquid (25) to cylinder valve through capillary tubes;
6. Monitor the color or pH of vent liquid;
7. Continue to clean until vent liquid become colorless of pH7;
8. After cleaning, change the vessel filled with dry chemical agent, and introduce dry chemical agent into cylinder valve;
9. After introducing of dry chemical agent, switch off the pump (24) and close valve 20;
10. Open valve 21 and introduce dry gas and purge the line until no liquid is observed at vent line (17);
11. If very short dry-down time is necessary, close valve 16, 21, and open valve 14, and evacuate cylinder valve by vacuum pump (19);
12. Close valve 14 and open valve 16, 21, and purge cylinder valve by dry gas;
13. Open valve 15 and close valve 16, and monitor moisture concentration in dry gas by hygrometer;
14. Continue to dry down cylinder valve by moisture concentration of < 1ppm;
15. Disconnect the connector (10) of apparatus and introduce of small amount of dry agent into cylinder valve, then put blind cap for cylinder valve.

An alternative embodiment of the present invention, which has the advantages of easier connection and operation automatism, is described in Fig. 1b. Here, the valve and connector parts which are exposed to air under conventional operation conditions of a gas cylinder are evacuated using an oil-free pump. The liquid cleaning agent and liquid drying agent respectively are introduced as a jet driven by the difference of the pressures surrounding the liquids (atmospheric pressure) and the one residing inside the valve and its connector parts.

On Fig. 1b, the following references have the following meaning:
101 to 110 are similar to respectively 1 to 10.
111. Cross type male connector
112. Dry gas (1.1-10 x 10⁵ Pa) inlet
113. Check valve
114. High pressure vessel
115. Cleaning liquid
116. Pressure gauge
117. Pneumatic two-way valve
118. Pneumatic three-way valve
119. Dry gas (1.1-10 x 10⁵ Pa) inlet
120. 0.1 *µ*m filter
121. Syringe
122. Dry chemical agent
123. Fine tube (inner diameter: 0.01-1mm)
124. Pneumatic two-way valve
125. Pneumatic three-way valve
126. Pneumatic two-way valve
127. Exhaust line of used cleaning liquid
128. Liquid trap
129. Used cleaning liquid
130. Valve for discarding used cleaning liquid
131. Vacuum assisted N₂ cycle purge line
132. Pneumatic two-way valve
133. Pneumatic three-way valve
134. Vacuum gauge
135. Oil-free vacuum pump

The operation of this apparatus on Fig. 1b is as follows:

### Wet-cleaning (washing) process

1. Close cylinder valve 101.
2. Put cleaning liquid into the high pressure vessel (114) and close the cap.
3. Introduce high pressure (1.1-10 x 10⁵ Pa) dry gas in the remaining space in the high pressure vessel (114) and check the pressure by the gauge (116).
4. Put dry chemical agent (122) in syringe (121).
5. Close the valve 117, 118, 124, 125, 126, 132 and 133.
6. Connect apparatus to cylinder valve outlet (108) by the connector (110).
7. Switch on pump (135) and open valve 133 and 125 to evacuate cylinder valve.
8. Evacuate cylinder valve by vacuum gauge shows below 5 x 10⁴ Pa, then close valve 125.
9. Open valve 117 and introduce pressurized (1.1-10 x 10⁵ Pa) cleaning liquid into cylinder valve.
10. After introducing cleaning liquid, close valve 117.
11. Maintain the cleaning liquid 0.01-15 min.
12. Open valve 125 and evacuate used cleaning liquid through the line (127) and evacuate cylinder valve (pump still running).
13. Evacuate cylinder valve until vacuum gauge shows below 5 x 10⁴ Pa, then close valve 125.
14. Repeat valve evacuation-cleaning liquid filling cycle (steps 9-13) more than one time (until used cleaning liquid becomes colorless or pH7).
15. After cleaning, close valve 117 and stop supplying cleaning liquid.
16. Evacuate cylinder valve through the line (127).
17. After the evacuation of valve, close 125 and 133.

### Wet-chemical drying process

18. After wet-cleaning, open valve 132 and 126 to evacuate cylinder valve.
19. After evacuation of cylinder valve, close valve 126.
20. Open the valve 118 and introduce dry gas of 1.1-10 x 10⁵ Pa into cylinder valve.
21. After introducing dry gas, close valve 118.
22. Open valve 126 and evacuate cylinder valve until vacuum gauge shows below 5 x 10⁴ Pa.
23. Repeat evacuation-dry gas filling cycle (steps 19-12) 1-10 times to remove remaining cleaning liquid in cylinder valve.
24. After above repeated cycle, close valve 118 and open valve 126 to evacuate cylinder valve.
25. After evacuation of cylinder valve, close valve 126.
26. Open valve 124 and introduce dry chemical agent (122) into cylinder valve through fine tube (123).
27. Keep filling dry chemical agent (122) in cylinder valve for 0.01-10 min.
28. Open valve 126 and evacuate cylinder valve until vacuum gauge shows below 5 x 10⁴ Pa.
29. Close valve 126.
30. Repeat evacuation-dry chemical agent filling cycle (steps 25-28) several (2-20) times to remove moisture in cylinder valve.
31. After above repeated cycle, close valve 124 and open valve 126 to evacuate cylinder valve.
32. After evacuation of cylinder valve, close valve 126.
33. Open valve 118 and introduce dry gas of 1.1-10 x 10⁵ Pa into cylinder valve.
34. After introducing dry gas, close valve 118.
35. Open valve 126 and evacuate cylinder valve until vacuum gauge shows below 5 x 10⁴ Pa.
36. Repeat evacuation-dry gas filling cycle (steps 32-35) more than 10 times to remove moisture and hydrocarbons in cylinder valve.
37. Repeat above cycle by moisture concentration of <1 ppm and hydrocarbon concentration of <100 ppb.
38. After above impurities reach the level, disconnect the connector (110) of apparatus with dry gas blowing from exit of connector (110) with opening valve 118, then put blind cap immediately.

Accordingly, the present invention provides a process for reducing corrosion in a gas distribution network of ultra high purity gas with minimized contamination and particulates. This process includes the use of a wet cleaning agent and a liquid drying the distribution network with a drying agent, to substantially remove the H₂O adsorbed to the gas communication surfaces of the gas distribution system as well as volatile and other impurities present in the network. The removal of adsorbed H₂O reduces undesirable reactions with the specialty gases that result in the generation of particulates, contaminants and corrosion.

Thereafter, the distribution network is purged with a dry gas having preferably a purity better than 1 ppm of each of any impurity, then it is evacuated and then exposed to either the ultra high purity corrosive gas or air, or both. The present invention thus provides an improved delivery of ultra high purity gases at the point of use, with minimized corrosion.

In order to further illustrate the present invention and the advantages thereof, the following specific examples are given, it being understood that same are intended only as illustrative and in nowise limitative.

### Example 1:

As an example of the present invention, HBr from a gas cylinder through a cylinder valve was analyzed.

Under conventional operating conditions using vacuum cycle purging, when the gas flows through a cylinder valve port and a short metal tubing for sampling, a very large particle count rate is observed as described in Figure 2. Also, the metallic surfaces of both the valve port and the tubing are visibly corroded, via formation of green or reddish superficial product growth. Chemical analysis reveals the formation of superficial iron-bromide hydrates. The above behavior is believed to be related to the presence of adsorbed moisture on the metallic parts exposed to air, which reacts with HBr to generate above corrosion and impurities in particulate form.

Improving the purge procedure of the line, using for instance a larger number of vacuum-pressure cycles, or increasing the HBr flow rate or flowing duration, decreases the extent of corrosion and the concentration of generated particulates as depicted in Figure 2.

In contrast, using the process of the present invention including wet cleaning with a wet cleaning agent at least inside of the valve and its outlet part, e.g. with DI water, or acetone or IPA, then liquid drying with an H₂O desorbing liquid drying agents, and then vacuum-purging of the residual gases after liquid drying, allows for essentially total absence of surface corrosion as well as the delivery of a contamination reduced and particulate reduced gas very shortly after the valve opening as depicted on the graph of Figures 3 and 4.

### Example 2:

The extent of corrosion of the cylinder valve can be measured precisely by applying a leaching methodology using DI water followed by chemical analysis of the rinsing solution. (Hattori et al., Jpn. J. Appl. Phys. 33, 2100 (1994) hereby incorporated by reference. The metal concentration in the leaching solution of constant volume is proportional to the extent of corrosion, i.e. of the volume of soluble corrosion products.

It is found by this method that high corrosion occurs when a valve has been used conventionally, i.e. flowing HBr gas after vacuum cycle purging of the cylinder connection when said cylinder valve was exposed to ambient atmosphere. However, when applying the process according to the invention, i.e. preliminary wet cleaning by DI water or IPA followed by liquid drying with an H₂O adsorbing liquid drying agent, corrosion on air exposure is essentially negligible and undetectable as depicted in the graph of Figure 4.

### Example 3:

Another commonly used corrosive gas is Dichlorosilane (DCS). A valve wherein DCS is flown after exposure of the valve to air and cylinder connection followed by vacuum cycle purging is very significantly corroded, as revealed by the metal leaching test (Fig. 5).

In contrast, if it is used with the invention, i.e. preliminary wet cleaning by DI water or IPA followed by liquid drying with an H₂O removing liquid drying agent and then flowing DCS for the same amount of time as above, corrosion is essentially undetectable (Fig. 5).

Various modifications and alterations of this invention will become apparent to those skilled in the art without departing from the scope of this invention as defined in the appended claims.

## Claims

1. A process for reducing corrosion in a gas distribution network of ultra high purity gas or any part of said distribution network, comprising:
(a) Wet cleaning the gas distribution network or at least one part thereof with a wet cleaning agent;
(b) Liquid drying said gas distribution network or said at least one part thereof with an H₂O desorbing liquid drying agent selected from the group consisting of acetone dimethylacetal DMP, 2.2 dichloropropane DCP or 2.2 dibromopropane DBP, mixtures thereof and any equivalent thereof;
(c) Purging said gas distribution network or any said part thereof with a dry high purity gas comprising less than 1 ppm of any impurity;
(d) Evacuating said gas distribution network or any said part thereof at a pressure which is lower than 5 x 10⁴ Pascal; and
(e) Exposing said gas distribution network or said any part thereof to an atmosphere comprising an ultra high purity corrosive gas or air.

2. The process according to Claim 1, wherein the step of wet cleaning is carried out for about 1 min. to about 1 hour.

3. The process according to Claim 2, using a distribution network of ultra high purity gas comprising essentially components or parts thereof which have never been used before, wherein said wet cleaning step is carried out for about 1 min. to about 2 min.

4. The process according to Claim 2, using a distribution network of ultra high purity gas comprising essentially components or parts thereof which have been used at least once before, wherein said wet cleaning step is carried out for about 5 to 30 minutes.

5. The process according to Claim 1, wherein the step (b) of liquid drying is carried out for about 1 min. to 20 min.

6. The process according to Claim 5, using a distribution network of ultra high purity gas comprising essentially components or parts thereof which have never been used before and having a roughness for their internal surface Ra which is lower than 5 x 10⁻⁶m, wherein said liquid drying step is carried out for about 1 to about 2 minutes.

7. The process according to Claim 5, using a distribution network of ultra high purity gas comprising essentially components or parts thereof which have been used at least once before wherein said liquid drying step is carried out for about 10 minutes or more.

8. The process according to Claim 5, using a distribution network of ultra high purity gas comprising essentially components or parts thereof which have a roughness of their internal surface Ra which is higher than 5 x 10⁻⁶m, wherein said liquid drying step is carried out for about 10 min. or more.

9. The process according to Claim 1, wherein said wet cleaning agent is a liquid comprising less than 1 mg. per liter of particulate material.

10. The process according to Claim 1, wherein said wet cleaning agent is a liquid comprising less than 10⁻⁶ g. per liter of particulate material.

11. The process according to Claim 1, wherein said wet cleaning agent is selected from the group comprising deionized water, isopropyl alcohol, acetone or mixture thereof.

12. The process according to Claim 1, further comprising repeating steps (a) and (b) before carrying out step (c).

13. The process according to Claim 1, further comprising purging the gas distribution network or any part thereof with an inert or reductive gas between steps (d) and (e).

14. The process according to Claim 13, wherein said inert or reductive gas is selected from the group comprising nitrogen, argon, helium or hydrogen.

15. The process according to Claim 13 or 14, wherein said inert or reductive gas comprises less than 100 ppb of volatile impurities and less than 1 particle per liter under standard conditions of temperature and pressure.

16. The process for distributing ultra high purity gases of Claim 1, wherein said gas distribution network includes at least one cylinder valve.

17. The process according to Claim 16, wherein said cylinder valve is submitted at least to step (a) and (b) before and after each contact of its internal surface with ambient air.

18. The process according to Claim 1, further comprising, during step (e), purging the gas distribution network or any part thereof with a high purity inert gas before exposing to ambient air the said gas distribution network or any part thereof.

## Patentansprüche

1. Verfahren zur Verminderung der Korrosion in einem Gasverteilungsnetz für ultrareines Gas oder einem Teil des Verteilungsnetzes, bei dem man:
(a) das Gasverteilungsnetz oder zumindest einen Teil davon mit einem Naßreinigungsmittel einer Naßreinigung unterwirft;
(b) das Gasverteilungsnetz oder den zumindest einen Teil davon mit einem H₂O desorbierenden flüssigen Trocknungsmittel aus der Gruppe bestehend aus Acetondimethylacetal DMP, 2,2-Dichlorpropan DCP oder 2,2-Dibrompropan DBP, deren Gemischen und jeglichem Äquivalent davon einer Flüssigtrocknung unterwirft;
(c) das Gasverteilungsnetz oder den Teil davon mit einem trockenen hochreinen Gas, das weniger als 1 ppm jeglicher Verunreinigung enthält, spült;
(d) das Gasverteilungsnetz oder den Teil davon bei einem Druck unter 5 x 10⁴ Pascal evakuiert und
(e) das Gasverteilungsnetz oder den Teil davon einer ein ultrareines korrosives Gas oder Luft enthaltenden Atmosphäre aussetzt.

2. Verfahren nach Anspruch 1, bei dem man den Naßreinigungsschritt für eine Dauer von etwa 1 Min. bis etwa 1 Stunde durchführt.

3. Verfahren nach Anspruch 2 unter Verwendung eines Gasverteilungsnetzes für ultrareines Gas, das im wesentlichen vorher noch nie verwendete Komponenten oder Teile davon enthält, bei dem man den Naßreinigungsschritt für eine Dauer von etwa 1 Min. bis etwa 2 Min. durchführt.

4. Verfahren nach Anspruch 2 unter Verwendung eines Gasverteilungsnetzes für ultrareines Gas, das im wesentlichen vorher mindestens einmal verwendete Komponenten oder Teile davon enthält, bei dem man den Naßreinigungsschritt für eine Dauer von etwa 5 bis etwa 30 Minuten durchführt.

5. Verfahren nach Anspruch 1, bei dem man den Flüssigtrocknungsschritt (b) für eine Dauer von etwa 1 Min. bis 20 Min. durchführt.

6. Verfahren nach Anspruch 5 unter Verwendung eines Gasverteilungsnetzes für ultrareines Gas, das im wesentlichen vorher noch nie verwendete und eine Innenoberflächenrauhigkeit Ra von weniger als 5 x 10⁻⁶ m aufweisende Komponenten oder Teile davon enthält, bei dem man den Flüssigtrocknungsschritt für eine Dauer von etwa 1 bis etwa 2 Minuten durchführt.

7. Verfahren nach Anspruch 5 unter Verwendung eines Gasverteilungsnetzes für ultrareines Gas, das im wesentlichen vorher mindestens einmal verwendete Komponenten oder Teile davon enthält, bei dem man den Flüssigtrocknungsschritt für eine Dauer von etwa 10 Minuten oder mehr durchführt.

8. Verfahren nach Anspruch 5 unter Verwendung eines Gasverteilungsnetzes für ultrareines Gas, das im wesentlichen eine Innenoberflächenrauhigkeit Ra von mehr als 5 x 10⁻⁶ m aufweisende Komponenten oder Teile davon enthält, bei dem man den Flüssigtrocknungsschritt für eine Dauer von etwa 10 Min. oder mehr durchführt.

9. Verfahren nach Anspruch 1, bei dem man als Naßreinigungsmittel eine Flüssigkeit mit weniger als 1 mg pro Liter teilchenförmigem Material einsetzt.

10. Verfahren nach Anspruch 1, bei dem man als Naßreinigungsmittel eine Flüssigkeit mit weniger als 10⁻⁶ g pro Liter teilchenförmigem Material einsetzt.

11. Verfahren nach Anspruch 1, bei dem man das Naßreinigungsmittel aus der Gruppe bestehend aus entionisiertem Wasser, Isopropylalkohol, Aceton und einem Gemisch davon auswählt.

12. Verfahren nach Anspruch 1, bei dem man ferner vor der Durchführung von Schritt (c) die Schritte (a) und (b) wiederholt.

13. Verfahren nach Anspruch 1, bei dem man ferner das Gasverteilungsnetz oder einen Teil davon zwischen den Schritten (d) und (e) mit einem inerten oder reduzierenden Gas spült.

14. Verfahren nach Anspruch 13, bei dem man das inerte oder reduzierende Gas aus der Gruppe bestehend aus Stickstoff, Argon, Helium und Wasserstoff auswählt.

15. Verfahren nach Anspruch 13 oder 14, bei dem das inerte oder reduzierende Gas weniger als 100 ppb flüchtige Verunreinigungen und weniger als 1 Teilchen pro Liter unter Normalbedingungen enthält.

16. Verfahren zur Verteilung von ultrareinen Gasen gemäß Anspruch 1, bei dem das Gasverteilungsnetz mindestens ein Zylinderventil aufweist.

17. Verfahren nach Anspruch 16, bei dem man das Zylinderventil vor und nach jedem Kontakt seiner Innenoberfläche mit Umgebungsluft mindestens Schritt (a) und Schritt (b) unterwirft.

18. Verfahren nach Anspruch 1, bei dem man ferner bei Schritt (e) das Gasverteilungsnetz oder einen Teil davon mit einem hochreinen Inertgas spült, bevor man das Gasverteilungsnetz oder einen Teil davon Umgebungsluft aussetzt.

## Revendications

1. Procédé de réduction de la corrosion dans un réseau de distribution de gaz d'un gaz à pureté ultra élevée ou dans une partie quelconque dudit réseau de distribution, comprenant :
(a) le nettoyage par voie humide du réseau de distribution de gaz ou d'au moins une partie de celui-ci à l'aide d'un agent de nettoyage par voie humide ;
(b) le séchage à liquide dudit réseau de distribution de gaz ou d'au moins ladite partie de celui-ci à l'aide d'un agent de séchage à liquide désorbant H₂O, choisi parmi le groupe se composant du diméthylacétal d'acétone DMP, du 2,2-dichloropropane DCP ou du 2,2-dibromopropane DBP, de mélanges de ces derniers ou d'un équivalent quelconque de ceux-ci ;
(c) la purge dudit réseau de distribution de gaz ou de toute dite partie de celui-ci à l'aide d'un gaz sec à pureté élevée, comprenant moins de 1 ppm d'une impureté quelconque ;
(d) l'évacuation dudit réseau de distribution de gaz ou d'une dite partie quelconque de celui-ci à une pression qui est inférieure à 5 x 10⁴ Pascal ; et
(e) l'exposition dudit réseau de distribution de gaz ou d'une dite partie quelconque de celui-ci à une atmosphère comprenant un gaz ou un air corrosif à pureté ultra élevée.

2. Procédé selon la revendication 1, **caractérisé en ce que** l'étape de nettoyage par voie humide est effectuée pendant une durée allant d'environ 1 minute à environ 1 heure.

3. Procédé selon la revendication 2, utilisant un réseau de distribution d'un gaz à pureté ultra élevée, comprenant pour l'essentiel des composants ou des pièces de celui-ci qui n'ont jamais été utilisés auparavant, **caractérisé en ce que** ladite étape de nettoyage par voie humide est effectuée pendant une durée d'environ 1 minute à environ 2 minutes.

4. Procédé selon la revendication 2, utilisant un réseau de distribution d'un gaz à pureté ultra élevée, comprenant pour l'essentiel des composants ou des pièces de celui-ci qui n'ont jamais été utilisés auparavant, **caractérisé en ce que** ladite étape de nettoyage par voie humide est effectuée pendant une durée d'environ 5 à environ 30 minutes.

5. Procédé selon la revendication 1, **caractérisé en ce que** l'étape (b) de séchage à liquide est effectuée pendant une durée d'environ 1 minute à environ 20 minutes.

6. Procédé selon la revendication 5, utilisant un réseau de distribution d'un gaz à pureté ultra élevée, comprenant pour l'essentiel des composants ou des pièces de celui-ci qui n'ont jamais été utilisés auparavant, et ayant une rugosité de leur surface interne Ra qui est inférieure à 5 x 10⁻⁶ m, **caractérisé en ce que** ladite étape de séchage à liquide est effectuée pendant une durée d'environ 1 à environ 2 minutes.

7. Procédé selon la revendication 5, utilisant un réseau de distribution d'un gaz à pureté ultra élevée, comprenant pour l'essentiel des composants ou des pièces de celui-ci qui ont été utilisés au moins une fois auparavant, **caractérisé en ce que** ladite étape de séchage à liquide est effectuée pendant une durée d'environ 10 minutes ou plus.

8. Procédé selon la revendication 5, utilisant un réseau de distribution d'un gaz à pureté ultra élevée comprenant pour l'essentiel des composants ou des pièces de celui-ci, qui ont une rugosité de leur surface interne Ra qui est supérieure à 5 x 10⁻⁶ m, **caractérisé en ce que** ladite étape de séchage à liquide est effectuée pendant une durée d'environ 10 minutes ou plus.

9. Procédé selon la revendication 1, **caractérisé en ce que** ledit agent de nettoyage par voie humide est un liquide comprenant moins de 1 mg par litre de matériau particulaire.

10. Procédé selon la revendication 1, **caractérisé en ce que** ledit agent de nettoyage par voie humide est un liquide comprenant moins de 10⁻⁶ g par litre de matière particulaire.

11. Procédé selon la revendication 1, **caractérisé en ce que** ledit agent de nettoyage par voie humide est choisi parmi le groupe comprenant l'eau déionisée, l'alcool isopropylique, l'acétone ou un mélange de ces derniers.

12. Procédé selon la revendication 1, comprenant en outre la répétition des étapes (a) et (b) avant l'exécution de l'étape (c).

13. Procédé selon la revendication 1, comprenant en outre la purge, entre les étapes (d) et (e), du réseau de distribution de gaz ou d'une partie quelconque de ce dernier, à l'aide d'un gaz inerte ou réducteur.

14. Procédé selon la revendication 13, **caractérisé en ce que** ledit gaz inerte ou réducteur est choisi parmi le groupe comprenant l'azote, l'argon, l'hélium ou l'hydrogène.

15. Procédé selon la revendication 13 ou la revendication 14, **caractérisé en ce que** ledit gaz inerte ou réducteur comprend moins de 100 ppb d'impuretés volatiles et moins de 1 particule par litre dans les conditions standard de température et de pression.

16. Procédé de distribution des gaz à pureté ultra élevée de la revendication 1, **caractérisé en ce que** ledit réseau de distribution de gaz comprend au moins une vanne de cylindre.

17. Procédé selon la revendication 16, **caractérisé en ce que** ladite vanne de cylindre est soumise au moins à l'étape (a) et à l'étape (b), avant et après chaque contact de sa surface interne avec l'air ambiant.

18. Procédé selon la revendication 1, comprenant en outre, pendant l'étape (e), la purge du réseau de distribution de gaz ou d'une partie quelconque de ce dernier à l'aide d'un gaz inerte à pureté élevée avant l'exposition à l'air ambiant dudit réseau de distribution de gaz ou d'une partie quelconque de ce dernier.
